# EUROPEAN PATENT SPECIFICATION

(11) **EP 2 610 333 B1**
(45) Date of publication and mention of the grant of the patent: **11.08.2021**
(21) Application number: 12197498.4
(22) Date of filing: 17.12.2012
(51) Int. Cl.: C10M 163/00, C10N 30/06, C10N 40/25, C10N 10/12

(54) **Fuel economical lubricating oil compositions for internal combustion engines**
Schmierölzusammensetzungen für Verbrennungsmotoren zur Treibstoffeinsparung
Compositions d'huile lubrifiante économique de carburant pour moteurs à combustion interne

(30) Priority: 27.12.2011 JP 2011286254
(43) Date of publication of application: 03.07.2013
(73) Proprietor: Chevron Japan Ltd., Tokyo 105-6218 (JP)
(72) Inventor: Ushioda, Nobuo, Omaezaki-shi, Shizuoka (JP); Ogasawara, Yasuhiro, Omaezaki-shi, Shizuoka (JP); Miyamoto, Tsuyoshi, Omaezaki-shi, Shizuoka (JP)
(74) Representative: Haseltine Lake Kempner LLP

(56) References cited:
- WO-A1-94/28095
- US-A1- 2008 167 207
- US-A1- 2008 248 981
- US-A1- 2011 021 393
- None

## Description

This application claims priority to Japanese Patent Application number JP2011-286254 which was filed in Japan on 12-27-2011.

### Field of Invention

The present invention relates to a lubricating oil composition which is favorably employable for lubricating internal combustion engines such as diesel engines, gasoline engines, and gas engines mounted on land-travelling vehicles, with high fuel economy.

### Background of Invention

Recently, the requirements for improvement of fuel economy to land-travelling vehicles on which a gasoline engine or a diesel engine is mounted, such as automotives, have continued with increased severity. It has been known that the improvement of fuel economy is most effectively made by reduction of weight of the vehicle on which an internal combustion engine is mounted. It also has been known that the improvement of fuel economy can be attained by appropriately selecting the lubricating oil composition employed for lubricating the internal combustion engine mounted on the vehicle.

For the reason described above, until now, the companies engaged for developing lubricating oil compositions as well as the companies engaged for developing lubricating oil additives have intensively made studies for providing lubricating oil compositions which show improved fuel economy.

The improvement of fuel economy provided by the lubricating oil composition generally can be attained by reduction of torque of rotation of the engine parts which is caused by the use of a lubricating oil composition providing reduction of friction to the sliding parts of the engine. The extent of reduction of friction provided by the lubricating oil composition mainly depends on the viscosity of the lubricating oil composition and selection of additives, mainly the selection of the friction modifier. For instance, if the lubricating oil composition is formulated with a base oil of low viscosity, the friction-reducing effect provided by the lubricating oil composition increases. However, the use of the base oil of low viscosity likely results in unfavorable phenomenon such as increase of oil consumption occurring during operation of the engine. Therefore, the improvement of fuel economy by the use of a lubricating oil composition employing a base oil of low viscosity has its limit. For this reason, intensive studies have been made on employment of appropriate lubricating oil additives, whereby improving the fuel economy provided by the lubricating oil composition. Until now, a variety of inventions made from these studies have been disclosed in a number of patent applications.

Patent publication 1 (JP 5-163497 A) discloses an engine oil composition showing low friction property, which comprises a base oil and an additive composition comprising a borated alkenylsuccinimide, an alkaline earth metal salicylate and molybdenum dithiophosphate and/or molybdenum dithiocarbamate.

Patent publication 2 (JP 6-336592 A) describes that a lubricating oil composition comprising zinc dialkyldithiophosphate being mainly composed of a zinc dialkyldithiophosphate having a secondary alkyl group, a metal-containing detergent composition comprising calcium sulfonate (e.g., TBN 200-300) and calcium salicylate (e.g., TBN 10-100), and molybdenum dithiocarbamate having a C₈₋₂₃ hydrocarbyl group shows increased low wear-producing property and increased low friction property.

Patent publication 3 (JP 8-302378 A) describes that an engine oil composition comprising a base oil having a specific kinematic viscosity and specific total aromatic content, an alkaline earth metal salicylate, zinc dialkyldithiophosphate, a succinimide ashless dispersant having a polybutenyl group having a molecular weight of 900-3500, a phenol type-ashless oxidation inhibitor, and molybdenum dithiocarbamate shows improved fuel economy. International publication WO94/28095 discloses lubricating oil compositions for internal combustion engines that reduce friction. The lubricating oil compositions contain molybdenum dithiocarbamate and a blend of a calcium salicylate and a calcium sulfonate detergent.

### Summary of Invention

The invention is defined in the appended claims.

Accordingly, it is the object of the invention to provide an improvement of a lubricating oil composition containing a molybdenum-containing friction modifier which is well known to give an excellent friction-reducing property as well as to improve the fuel economy. The improved lubricating oil composition of the invention shows further increased fuel economy.

The inventors of the present invention have studied on the synergistic effects for improvement of fuel economy provided by combinations of the molybdenum-containing friction modifier and various lubricating oil additives. As a result of the studies, the inventors have found that a lubricating oil composition containing a combination of the molybdenum-containing friction modifier and an overbased metal-containing detergent composition comprising calcium salicylate having an alkyl group having an average carbon atom number of 14-18 (at least 60 mol.% of the alkyl group has a carbon atom number of 14-18), and calcium sulfonate having an alkyl group having an average carbon atom number of 20-24 (at least 60 mol.% of the alkyl group has a carbon atom number of 20-24), and/or calcium salicylate having an alkyl group having an average carbon atom number of 20-28 (at least 60 mol.% of the alkyl group has a carbon atom number of 20-28) shows surprisingly improved fuel economy. The invention described herein has been made on this finding.

Accordingly, the present invention provides a lubricating oil composition for internal combustion engines which comprises a major amount of an oil of lubricating viscosity and a minor amount of an additive composition comprising an overbased metal-containing detergent composition and a molybdenum-containing friction modifier,
wherein the overbased metal-containing detergent composition comprises calcium salicylate having an alkyl group having an average carbon atom number in the range of 14 to 18, at least 60 mol.% (preferably, at least 70 mol.%) of said alkyl group having a carbon atom number in the range of 14 to 18; and at least one of the following calcium-containing detergents:
calcium sulfonate having an alkyl group having an average carbon atom number in the range of 20 to 24, at least 60 mol.% (preferably, at least 70 mol.%) of said alkyl group having a carbon atom number in the range of 20 to 24, and
calcium salicylate having an alkyl group having an average carbon atom number in the range of 20 to 28, at least 60 mol.% (preferably, at least 70 mol.%) of said alkyl group having a carbon atom number in the range of 20 to 28.

The lubricating oil composition of the invention contains the base oil (i.e., oil of lubricating viscosity) generally in the amount of 70 wt.% or more, preferably in the amount of 80 wt.% or more, of the lubricating oil composition.

### Detailed Description of Invention

Preferred embodiments of the invention are described below.
(1) The molybdenum-containing friction modifier comprises molybdenum dithiocarbamate.
(2) The calcium salicylate having an alkyl group having an average carbon atom number in the range of 14 to 18, at least 60 mol.% of said alkyl group having a carbon atom number in the range of 14 to 18 has an overbased degree of 1 to 4, and the calcium sulfonate having an alkyl group having an average carbon atom number in the range of 20 to 24, at least 60 mol.% of said alkyl group having a carbon atom number in the range of 20 to 24 and the calcium salicylate having an alkyl group having an average carbon atom number in the range of 20 to 28, at least 60 mol.% of said alkyl group having a carbon atom number in the range of 20 to 28 have an overbased degree of 6 to 24.
(3) A ratio of the overbased degree of the calcium sulfonate having an alkyl group having an average carbon atom number in the range of 20 to 24, at least 60 mol.% of said alkyl group having a carbon atom number in the range of 20 to 24 and the calcium salicylate having an alkyl group having an average carbon atom number in the range of 20 to 28, at least 60 mol.% of said alkyl group having a carbon atom number in the range of 20 to 28 to the calcium salicylate having an alkyl group having an average carbon atom number in the range of 14 to 18, at least 60 mol.% of said alkyl group having a carbon atom number in the range of 14 to 18 is in the range of 2 to 12.
(4) The overbased metal-containing detergent composition comprises the calcium salicylate having an alkyl group having an average carbon atom number in the range of 14 to 18, at least 60 mol.% of said alkyl group having a carbon atom number in the range of 14 to 18 and the calcium sulfonate having an alkyl group having an average carbon atom number in the range of 20 to 24, at least 60 mol.% of said alkyl group having a carbon atom number in the range of 20 to 24.
(5) The overbased metal-containing detergent composition comprises the calcium salicylate having an alkyl group having an average carbon atom number in the range of 14 to 18, at least 60 mol.% of said alkyl group having a carbon atom number in the range of 14 to 18 and the calcium salicylate having an alkyl group having an average carbon atom number in the range of 20 to 28, at least 60 mol.% of said alkyl group having a carbon atom number in the range of 20 to 28.
(6) The lubricating oil composition comprises the molybdenum-containing friction modifier in an amount of 0.01 to 0.15 wt.% in terms of molybdenum content in the lubricating oil composition.
(7) The lubricating oil composition comprises each of the calcium salicylate having an alkyl group having an average carbon atom number in the range of 14 to 18, at least 60 mol.% of said alkyl group having a carbon atom number in the range of 14 to 18 and at least one of the following calcium-containing detergents: calcium sulfonate having an alkyl group having an average carbon atom number in the range of 20 to 24, at least 60 mol.% of said alkyl group having a carbon atom number in the range of 20 to 24 and calcium salicylate having an alkyl group having an average carbon atom number in the range of 20 to 28, at least 60 mol.% of said alkyl group having a carbon atom number in the range of 24 to 28 in an amount of 0.01 to 0.4 wt.% in terms of calcium content in the lubricating oil composition.
(8) The lubricating oil composition further comprises a low overbased calcium sulfonate having an alkyl group having an average carbon atom number in the range of 14 to 24, at least 60 mol.% of said alkyl group having a carbon atom number in the range of 14 to 24 and having an overbased degree of 0.1 to 2.
(9) The lubricating oil composition further comprises a lubricating oil additive selected from the group consisting of a nitrogen-containing ashless dispersant, a zinc phosphate oxidation inhibitor, a zinc phosphate anti-wear agent, a phenolic oxidation inhibitor, and an amine oxidation inhibitor.
(10) Each of the zinc phosphate oxidation inhibitor and zinc phosphate anti-wear agent comprises a mixture of zinc di(primary alkyl) dithiophosphate and zinc di(secondary alkyl) dithiophosphate in a weight ratio of 1/9 to 9/1.
(11) The nitrogen-containing ashless dispersant is a succinimide dispersant which may be post-treated with ethylene carbonate or a borate compound.
(12) The lubricating oil composition further comprises a molybdenum complex of succinimide which may contain sulfur.
(13) The oil of lubricating viscosity has a viscosity index of 120 to 160.
(14) The lubricating oil composition satisfies SAE viscosity grade of 0W20.

The lubricating oil composition of the invention provides increased high fuel economy to internal combustion engines such as gasoline engines and diesel engines. Therefore, vehicles on which these internal combustion engines are mounted show improved fuel economy.

The base oil and additives employable for the preparation of the lubricating oil composition of the invention are described below in more detail.

### Base oil

The base oil (i.e., oil of lubricating viscosity) generally is a mineral oil or a synthetic oil showing a kinematic viscosity of 2 to 50 mm²/s at 100°C. There are no specific limitations on the natures and other properties of the mineral oil and synthetic oil. However, the sulfur content of the base oil should be 0.1 wt.% or less. The sulfur content preferably is 0.03 wt.% or less, and more preferably is 0.005 wt.% or less.

The mineral oil preferably is an oil which is obtained by processing a lubricating oil distillate of a mineral oil by solvent refining, hydrogenation, or their combination. Particularly preferred is a highly hydrogenated refined oil (corresponding to a hydrocracked oil, typically has a viscosity index of 120 to 160, an aromatic component content of 5 wt.% or less, a nitrogen content of 50 wt.ppm or less, and a sulfur content of 50 wt. ppm or less). Particularly preferred is a high viscosity index base oil, for instance, a base oil having a viscosity index of 140 to 160 which is obtained by hydroisomerization of slack wax or GTL wax (Gas-To-Liquid).

Examples of the synthetic oils (synthetic lubricating base oils) include poly-□-olefin such as a polymerized compound of □-olefin having 3 to 12 carbon atoms; a dialkyl ester of a di-basic acid such as sebacic acid, azelaic acid or adipic acid and an alcohol having 4 to 18 carbon atoms, typically dioctyl sebacate; a polyol ester which is an ester of 1,1,1-trimethylolpropane or pentaerythritol and a mono-basic acid having 3 to 18 carbon atoms; and alkylbenzene having an alkyl group of 9 to 40 carbon atoms. The synthetic oil generally contains essentially no sulfur, shows good stability to oxidation and good heat resistance, and gives less residual carbon and soot when it is burned. Therefore, the synthetic oil is preferably employed for the lubricating oil composition of the invention. Particularly preferred is poly-□-olefin, from the viewpoint of the object of the invention.

Each of the mineral oil and synthetic oil can be employed singly. If desired, however, two or more mineral oils can be employed in combination, and two or more synthetic oils can be employed in combination. The mineral oil and synthetic oil can be employed in combination at an optional ratio.

### Molybdenum-containing friction modifier

The lubricating oil composition of the invention contains a molybdenum-containing friction modifier. The molybdenum-containing friction modifier can be any one of the known molybdenum-containing friction modifiers or the known molybdenum-containing friction modifier compositions. These friction modifiers and friction modifier compositions are described in the aforementioned Patent publications 1 to 3.

Preferred molybdenum-containing friction modifier is, for example, sulfurized oxymolybdenum dithiocarbamate, sulfurized oxymolybdenum dithiophosphate, amine-molybdenum complex compound, oxymolybdenum diethylate amide, and oxymolybdenum monoglyceride. Most preferred is a molybdenum dithiocarbamate friction modifier.

The lubricating oil composition of the invention generally contains the molybdenum-containing friction modifier in an amount of 0.01 to 0.15 wt.% in terms of the molybdenum content.

### Overbased metal-containing detergent

The lubricating oil composition of the invention contains a combination of the following overbased metal-containing detergents:
(a) calcium salicylate (specifically, monoalkylsalicylate) having an alkyl group having an average carbon atom number in the range of 14 to 18, at least 60 mol.% of said alkyl group having a carbon atom number in the range of 14 to 18; and
(b) calcium sulfonate (specifically, monoalkylsulfonate) having an alkyl group having an average carbon atom number in the range of 20 to 24, at least 60 mol.% of said alkyl group having a carbon atom number in the range of 20 to 24, and/or calcium salicylate (specifically, monoalkylsalicylate) having an alkyl group having an average carbon atom number in the range of 20 to 28, at least 60 mol.% of said alkyl group having a carbon atom number in the range of 20 to 28.

Each of the above-mentioned components (b), namely, calcium sulfonate having an alkyl group having an average carbon atom number in the range of 20 to 24, at least 60 mol.% of said alkyl group having a carbon atom number in the range of 20 to 24, and calcium salicylate having an alkyl group having an average carbon atom number in the range of 20 to 28, at least 60 mol.% of said alkyl group having a carbon atom number in the range of 20 to 28 can be employed singly or in combination.

The above-mentioned component (a), namely, calcium salicylate having an alkyl group having an average carbon atom number in the range of 14 to 18, at least 60 mol.% of said alkyl group having a carbon atom number in the range of 14 to 18 preferably is a mixture comprising plural calcium salicylates having an alkyl group having an average carbon atom number in the range of 14 to 18 in an amount of 60 mol.% or more, particularly 70 mol.% or more.

One of the above-mentioned component (b), namely, calcium sulfonate having an alkyl group having an average carbon atom number in the range of 20 to 24, at least 60 mol.% of said alkyl group having a carbon atom number in the range of 20 to 24 preferably is a mixture comprising plural calcium sulfonates having an alkyl group having an average carbon atom number in the range of 20 to 24 in an amount of 60 mol.% or more, particularly 70 mol.% or more.

Another of the above-mentioned component (b), namely, calcium salicylate having an alkyl group having an average carbon atom number in the range of 20 to 28, at least 60 mol.% of said alkyl group having a carbon atom number in the range of 20 to 28 preferably is a mixture comprising plural calcium salicylates having an alkyl group having an average carbon atom number in the range of 20 to 28 in an amount of 60 mol.% or more, particularly 70 mol.% or more.

The lubricating oil composition contains each of the component (a) and component (b) generally in an amount of 0.01 to 0.4 wt.%, in terms of calcium content, based on the total amount of the lubricating oil composition.

It is preferred that the calcium salicylate of the component (a) is calcium salicylate having an overbased degree of 1 to 4, particularly 1.5 to 3. The calcium salicylate can be sulfurized or unsulfurized.

It is preferred that the calcium sulfonate and calcium salicylate of the component (b) are calcium sulfonate and calcium salicylate independently having an overbased degree of 6 to 24. Preferably, the calcium sulfonate has an overbased degree of 14 to 20, and the calcium salicylate has an overbased degree of 6 to 12.

The ratio of overbased degree for the component (b)/component (a) is preferably in the range of 2 to 12.

It is preferred that the lubricating oil composition of the invention further contains calcium sulfonate having an alkyl group having an average carbon atom number in the range of 14 to 24, at least 60 mol.% (preferably, at least 70 mol.%) of said alkyl group having a carbon atom number in the range of 14 to 24 and having an overbased degree of 0.1 to 2.

The lubricating oil composition of the invention can further contain relatively small amounts of other overbased or less overbased metal-containing detergents than the above-mentioned components (a) and (b). These metal-containing detergents may be salicylates, carboxylates, sulfonates and/or phenates.

### Other additives

The lubricating oil composition of the invention can further contain other lubricating oil additives. Examples of the other lubricating oil additives include nitrogen-containing ashless dispersants, zinc phosphate oxidation inhibitors (or zinc phosphate anti-wear agent) such as zinc dihydrocarbyldithiophosphate, and organic oxidation inhibitors (e.g., phenolic oxidation inhibitors and amine oxidation inhibitors).

The nitrogen-containing ashless dispersant preferably is an alkenyl- or alkyl-succinimide derived from polyolefin or a derivative thereof. The lubricating oil composition can contain the nitrogen-containing ashless dispersant in an amount of 0.01 to 0.3 wt.%, in terms of the nitrogen content, based on the amount of the lubricating oil composition. A representative succinimide can be prepared by the reaction between succinic anhydride substituted with a high molecular weight alkenyl or alkyl and a polyalkylene polyamine containing average 4 to 10 (preferably 5 to 7) nitrogen atoms in one molecule. The high molecular weight alkenyl or alkyl is preferably derived from polybutene having a number average molecular weight of about 900 to 3,000.

The process for obtaining the polybutenyl-succinic anhydride by the reaction of polybutene and maleic anhydride is generally performed by the chlorination process using a chloride compound. Otherwise, a thermal reaction process using no chlorine compound can be employed. It is preferred to employ a polybutenylsuccinimide which is derived from a polybutenylsuccinic anhydride by the thermal reaction process.

The succinimide can be a post-treated succinimide which is prepared by the reaction with boric acid, alcohol, aldehyde, ketone, alkylphenol, cyclic carbonate, organic acid or the like. Particularly, a borated alkenyl(or alkyl)-succinimide which is obtained by the reaction with a boron-containing compound such as boric acid or a boron compound is advantageous from the viewpoints of thermal and oxidation stability.

The lubricating oil composition may contain other ashless dispersants such as an alkenylbenzylamine ashless dispersant and/or an alkenylsuccinic acid ester ashless dispersant in addition to or in place of the above-mentioned alkenyl(or alkyl)-succinimide ashless dispersant.

The lubricating oil composition may contain a zinc phosphate oxidation inhibitor (or zinc phosphate anti-ware agent). The zinc phosphate oxidation inhibitor (or zinc phosphate anti-ware agent) may be selected from the group consisting of zinc dialkyldithiophosphate, zinc di-alkylmonothiophosphate and zinc dihydrocarbylphosphate). The zinc phosphate oxidation inhibitors/anti-wear agents are well known with respect to their preparation processes and natures. The zinc phosphate oxidation inhibitors/anti-wear agents are generally contained in an amount of 0.01 to 0.12 wt.%, in terms of the phosphorus content, based on the amount of the lubricating oil composition. However, the amount preferably is in the range of 0.01 to 0.06 wt.%, in consideration of the preparation of a low-phosphorus, low-sulfur lubricating oil composition.

The zinc dialkyldithiophosphate preferably contains an alkyl group having 3-18 carbon atoms or an alkylaryl group having C₃₋₁₈ alkyl group. Most preferred is a zinc dialkyldithiophosphate containing an alkyl group derived from a secondary alcohol having 3-18 carbon atoms or a zinc dialkyldithiophosphate containing a mixture of alkyl groups derived from a mixture of a primary alcohol having 3-18 carbon atoms and a secondary alcohol having 3-18 carbon atoms. Both are particularly effective for reducing wear. A zinc dialkyldithiophosphate derived from a primary alcohol shows high thermal resistance. These zinc dialkyldithiophosphates can be employed alone or in combination in the form of a mixture mainly comprising one derived from the secondary alcohol and/or one derived from the primary alcohol.

The lubricating oil composition of the invention preferably contains an organic oxidation inhibitor in an amount of 0.01-5 wt.%, preferably 0.1-3 wt.%. The oxidation inhibitor can be a hindered phenol oxidation inhibitor or a diarylamine oxidation inhibitor. The diarylamine oxidation inhibitor is advantageous in giving a base number originating from the nitrogen atoms. The hindered phenol oxidation inhibitor is advantageous in producing no NOₓ gas.

Examples of the hindered phenol oxidation inhibitors include 2,6-di-t-butyl-p-cresol, 4,4'-methylenebis(2,6-di-t-butylphenol), 4,4'-methylenebis(6-t-butyl-o-cresol), 4,4'-isopropylidenebis(2,6-di-t-butylphenol), 4,4'-bis(2,6-di-t-butylphenol), 2,2'-methylenebis(4-methyl-6-t-butylphenol), 4,4'-thiobis(2-methyl-6-t-butylphenol), 2,2-thio-diethylenebis[3-(3,5-dit-butyl-4-hydoxyphenyl)propionate], octyl 3-(3,5-di-t-butyl-4-hydroxyphenyl)propionate, octadecyl 3-(3,5-di-t-butyl-4-hydroxyphenyl)propionate, and octyl 3-(3,5-t-butyl-4-hydroxy-3-methylphenyl)propionate.

Examples of the diarylamine oxidation inhibitors include alkyldiphenylamine having a mixture of alkyl groups of 4 to 9 carbon atoms, p,p'-dioctyldiphenylamine, phenyl-□-naphthylamine, phenyl-□-naphthylamine, alkylated □-naphthylamine, and alkylated phenyl-□-naphthylamine.

Each of the hindered phenol oxidation inhibitor and diarylamine oxidation inhibitor can be employed alone or in combination. If desired, other oil soluble oxidation inhibitors can be employed in combination with the above-mentioned oxidation inhibitor(s).

The lubricating oil composition of the invention may further contain an oxymolybdenum complex of succinimide, particularly a sulfur-containing oxymolybdenum complex of succinimide. The sulfur-containing oxymolybdenum complex of succinimide can provide increased oxidation inhibition when it is employed in combination with the above-mentioned phenolic or amine oxidation inhibitors.

The lubricating oil composition of the invention may further contain an alkali metal borate hydrate in an amount of 5 wt.% or less, particularly in an amount of 0.01 to 5 wt.%. A representative alkali metal borate hydrate can be prepared in the manner described in United States Patents 3,929,650 and 4,089,790. For example, the alkali metal borate hydrate can be in the form of a dispersion containing micro-particles of an alkali metal borate hydrate which is produced by carbonizing a neutral alkali metal or alkaline earth metal sulfonate in the presence of an alkali metal hydroxide to yield an overbased sulfonate and reacting the overbased sulfonate with boric acid. In the carbonizing procedure, it is desired to incorporate an ashless dispersant such as succinimide into the reaction mixture. The alkali metal preferably is potassium or sodium. The alkali metal borate hydrate can be a dispersion of KB₃O₅□H₂O particles having a particle size of about 0.3 □m or less which is dispersed in the presence of a neutral calcium sulfonate and succinimide.

The lubricating oil composition of the invention preferably contains a viscosity index improver in an amount of 20 wt.% or less, preferably 1 to 20 wt.%. Examples of the viscosity index improvers are polymers such as polyalkyl methacrylate, ethylene-propylene copolymer, styrene-butadiene copolymer, and polyisoprene. A dispersant viscosity index improver and a multi-functional viscosity index improver which are produced by providing dispersing properties to the above-mentioned polymer are preferably employed. The viscosity index improvers can be used alone or in combination.

The lubricating oil composition of the invention may further contain a small amount of various auxiliary additives. Examples of the auxiliary additives are described below.

Oxidation inhibitor or anti-wear agent such as zinc dithiocarbamate, methylenebis(dibutyldithiocarbamate), oil soluble copper compounds, sulfur-containing compounds (e.g., sulfurized olefins, sulfurized esters, and polysulfide), phosphoric acid esters, phosphorous acid esters, thiophosphoric acid esters, and organic amide compounds (e.g., oleylamide); benzotriazol compounds and thiadiazol compounds functioning as metal deactivating agent; and nonionic polyoxyalkylene surface active agents such as polyoxyethylenealkylphenyl ether and copolymers of ethylene oxide and propylene oxide functioning as an antirust agent and an anti-emulsifying agent.

Further, various amines, amides, amine salts and their derivatives which can function as friction modifiers can be employed.

Furthermore, various compounds functioning as an anti-foaming agent and a pour point depressant can be incorporated.

The above-mentioned auxiliary additives may be incorporated into the lubricating oil composition in an amount of 3 wt.% or less, particularly in an amount of 0.001-3 wt.%.

### Examples [1-3], and Comparative Examples [1-3]

### (1) Preparation of lubricating oil compositions (test oils)

Lubricating oil compositions were prepared by adding the below-mentioned additive components to the base oil to give the formulations set forth in Table 1. The lubricating oil compositions of Examples 1 to 3 are according to the invention, while the lubricating oil compositions of Comparative Examples 1 to 3 are for comparison. The lubricating oil compositions were formulated to show a viscosity grade (SAE viscosity grade) of 0W20 and a kinematic viscosity of 7.7-7.8 mm²/s at 100°C, by addition of a viscosity index improver.

### (2) Base oil and additives

### (I)Base oil:

Mineral base oil (kinematic viscosity at 100°C: 4.1 mm²/s, viscosity index: 137) prepared from slack wax via hydrogenation, fractional distillation and dewaxing.

### (II) Additives

### Nitrogen-containing ashless dispersant

Ethylene carbonate post-treated succinimide dispersant (bis-type, nitrogen content: 1.0 wt.%) derived from polybutene (number average molecular weight: about 2,300).

### Metal-containing detergent

a) Overbased Ca salicylate (1)[Ca-sali-1]: Calcium monoalkylsalicylate having alkyl groups in which approx. 80 mol.% of the whole alkyl groups were C₁₄₋₁₈ alkyl groups (Ca: 6.1 wt.%, S: 0.1 wt.%, TBN: 170 mg KOH/g, overbased degree: 2.3)
b) Overbased Ca sulfonate [Ca-sulf-1]: Calcium alkyltoluenesulfonate having alkyl groups in which approx. 80 mol.% of the whole alkyl groups were C₂₀₋₂₄ alkyl groups (Ca: 16.0 wt.%, S: 1.6 wt.%, TBN: 423 mg KOH/g, overbased degree: 17)
c) Overbased Ca salicylate (2)[Ca-sali-2]: Calcium monoalkylsalicylate having alkyl groups in which approx. 80 mol.% of the whole alkyl groups were C₂₀₋₂₈ alkyl groups (Ca: 11.4 wt.%, S: 0.2 wt.%, TBN: 320 mg KOH/g, overbased degree: 8.2)
d) Low overbased Ca sulfonate [Ca-sulf-2]: Calcium alkylbenzenesulfonate having alkyl groups in which approx. 80 mol.% of the whole alkyl groups were C₁₄₋₂₄ alkyl groups (Ca: 2.4 wt.%, S: 2.9 wt.%, TBN: 17 mg KOH/g, overbased degree: 0.34)

### Molybdenum-containing friction modifier

Sulfurized oxymolybdenum dithiocarbamate (Mo-DTC, Mo: 10 wt.%, S: 11 wt.%)

### Zinc phosphate oxidation inhibitor

Zinc di(secondary alkyl)dithiophosphate (ZnDTP-1, P: 7.8 wt.%, Zn: 7.8 wt.%, S: 14 wt.%)

Zinc di(primary alkyl)dithiophosphate (ZnDTP-2, P: 7.3 wt.%, Zn: 8.4 wt.%, S: 14 wt.%)

### Organic oxidation inhibitor(Ox. Inhi.

Amine oxidation inhibitor: dialkyldiphenylamine

### Sulfur-containing succinimide-molybdenum complex (Mo comp.)

Mo-containing complex (Mo: 5.5 wt.%, S: 0.2 wt.%, N: 1.6 wt.%, TBN: 10 mg KOH/g)

### Viscosity index improver

Polymethacrylate viscosity index improver

### (3) Evaluation of lubricating oil compositions

### a) Test method

The crank shaft of a gasoline engine (in-line 4 cylinder engine, engine swept volume: 1.8 L, roller type-valve system) was rotated by means of an electric motor connected via a torque meter, and the running torque was monitored. In advance of starting the test, the ignition plug was removed so as to minimize the effect caused by pumping loss of the pistons, and the test was carried out under open conditions. The oil temperature was kept to 100°C. The test was carried out at respective rotational rates for 150 seconds. The torques were continuously monitored during the period from the time at a lapse of 30 sec. from the beginning of the test to 120 sec. An average torque value was calculated from the monitored torque values.

Independently, a reference oil (SAE viscosity grade: 0W20, kinematic viscosity at 100°C: 8.9 mm²/s) was prepared.

From the torque value and the above-mentioned average torque value of the tested oil, a torque reduction ratio (%) was calculated. The torque reduction ratio is set forth in Table 1.

### b) Test results

The test results of the test oils are set forth in Table 1 below.

**Table 1**

| Additives | Ex.1 | Ex.2 | Ex.3 | Com.1 | Com.2 | Com.3 |
|---|---|---|---|---|---|---|
| Ashless | | | | | | |
| Dispersant | 0.03 | 0.03 | 0.03 | 0.03 | 0.03 | 0.03 |
| Ca-sali-1 | 0.12 | 0.06 | 0.12 | 0.18 | - | - |
| Ca-sul-1 | 0.06 | 0.12 | - | - | 0.18 | - |
| Ca-sali-2 | - | - | 0.06 | - | - | 0.18 |
| Ca-sul-2 | 0.02 | 0.02 | 0.02 | 0.02 | 0.02 | 0.02 |
| Mo-DTC | 0.07 | 0.07 | 0.07 | 0.07 | 0.07 | 0.07 |
| ZnDTP-1 | 0.03 | 0.03 | 0.03 | 0.03 | 0.03 | 0.03 |
| ZnDTP-2 | 0.05 | 0.05 | 0.05 | 0.05 | 0.05 | 0.05 |
| Ox.inhi. | 1.2 | 1.2 | 1.2 | 1.2 | 1.2 | 1.2 |
| Mo.comp. | 0.4 | 0.4 | 0.4 | 0.4 | 0.4 | 0.4 |

In Table 1, Ex. = Example; Com. = Comparative Example

### Test results

| Torque reduction ratio (%) | | | | | | |
|---|---|---|---|---|---|---|
| 550 rpm | 6.2 | 5.9 | 6.0 | 5.5 | 5.3 | 5.7 |
| 950 rpm | 4.2 | 4.2 | 3.9 | 3.5 | 3.7 | 3.6 |
| 1500 rpm | 2.0 | 2.2 | 2.0 | 1.6 | 1.9 | 1.3 |

### Remarks:

The amounts of the additives are indicated as follows:
Ox.inhi. (i.e., organic oxidation inhibitor) and Mo.comp. (i.e., sulfur-containing succinimide-molybdenum complex) are set forth in terms of the amount (wt.%) of the additive *per se;*
Ashless additive, calcium-containing detergents (Ca-sali-1, Ca-sul-1, Ca-sali-2, Ca-sul-2), Mo-DTC, and Zinc-containing compounds (ZnDTP-1, ZnDTP-2) are set forth in terms of N content (wt.%), Ca content (wt.%), Mo content (wt.%), and P content (wt.%), respectively.

The test results set forth in Table 1 indicate that the lubricating oil composition according to the invention (Examples 1 to 3) show extremely high torque reduction as compared with the lubricating oil compositions (Comparison Examples 1 to 3) containing metal-containing detergents differing from those contained in the lubrication oil compositions of Examples 1 to 3.

## Claims

1. A lubricating oil composition for internal combustion engines which comprises a major amount of an oil of lubricating viscosity and a minor amount of an additive composition comprising an overbased metal-containing detergent composition and a molybdenum-containing friction modifier;
wherein the overbased metal-containing detergent composition comprises 0.01 to 0.4 wt.%, in terms of calcium content, based on the total amount of the lubricating oil composition, of a calcium salicylate having an alkyl group having an average carbon atom number in the range of 14 to 18, at least 60 mol.% of said alkyl group having a carbon atom number in the range of 14 to 18, wherein the calcium salicylate is a mixture of a plurality of calcium salicylates;
and 0.01 to 0.4 wt.%, in terms of calcium content, based on the total amount of the lubricating oil composition, of at least one of the following calcium-containing detergent:
calcium sulfonate having an alkyl group having an average carbon atom number in the range of 20 to 24, at least 60 mol.% of said alkyl group having a carbon atom number in the range of 20 to 24, wherein the calcium sulfonate is a mixture of a plurality of calcium sulfonates; and
calcium salicylate having an alkyl group having an average carbon atom number in the range of 20 to 28, at least 60 mol.% of said alkyl group having a carbon atom number in the range of 20 to 28, wherein the calcium salicylate is a mixture of a plurality of calcium salicylates.

2. The lubricating oil composition of claim 1, wherein the molybdenum-containing friction modifier comprises molybdenum dithiocarbamate.

3. The lubricating oil composition of claim 1, wherein the calcium salicylate having an alkyl group having an average carbon atom number in the range of 14 to 18, at least 60 mol.% of said alkyl group having a carbon atom number in the range of 14 to 18 has an overbased degree of 1 to 4, and the calcium sulfonate having an alkyl group having an average carbon atom number in the range of 20 to 24, at least 60 mol.% of said alkyl group having a carbon atom number in the range of 20 to 24 and the calcium salicylate having an alkyl group having an average carbon atom number in the range of 20 to 28, at least 60 mol.% of said alkyl group having a carbon atom number in the range of 20 to 28 have an overbased degree of 6 to 24.

4. The lubricating oil composition of claim 3, wherein the ratio of the overbased degree of the calcium sulfonate having an alkyl group having an average carbon atom number in the range of 20 to 24, at least 60 mol.% of said alkyl group having a carbon atom number in the range of 20 to 24 and the calcium salicylate having an alkyl group having an average carbon atom number in the range of 20 to 28, at least 60 mol.% of said alkyl group having a carbon atom number in the range of 20 to 28 to the calcium salicylate having an alkyl group having an average carbon atom number in the range of 14 to 18, at least 60 mol.% of said alkyl group having a carbon atom number in the range of 14 to 18 is in the range of 2 to 12.

5. The lubricating oil composition of claim 1, wherein the overbased metal-containing detergent comprises the calcium salicylate having an alkyl group having an average carbon atom number in the range of 14 to 18, at least 60 mol.% of said alkyl group having a carbon atom number in the range of 14 to 18 and the calcium sulfonate having an alkyl group having an average carbon atom number in the range of 20 to 24, at least 60 mol.% of said alkyl group having a carbon atom number in the range of 20 to 24.

6. The lubricating oil composition of claim 1, wherein the overbased metal-containing detergent composition comprises the calcium salicylate having an alkyl group having an average carbon atom number in the range of 14 to 18, at least 60 mol.% of said alkyl group having a carbon atom number in the range of 14 to 18 and the calcium salicylate having an alkyl group having an average carbon atom number in the range of 20 to 28, at least 60 mol.% of said alkyl group having a carbon atom number in the range of 20 to 28.

7. The lubricating oil composition of claim 1, which comprises the molybdenum-containing friction modifier in an amount of 0.01 to 0.15 wt.% in terms of molybdenum content in the lubricating oil composition.

8. The lubricating oil composition of claim 1, which further comprises a low overbased calcium sulfonate having an alkyl group having an average carbon atom number in the range of 14 to 24, at least 60 mol.% of said alkyl group having a carbon atom number in the range of 14 to 24 and having an overbased degree of 0.1 to 2.

9. The lubricating oil composition of claim 1, which further comprises a lubricating oil additive selected from the group consisting of a nitrogen-containing ashless dispersant, a zinc phosphate oxidation inhibitor, a zinc phosphate wear inhibitor, a phenolic oxidation inhibitor, and an amine oxidation inhibitor.

10. The lubricating oil composition of claim 9, wherein each of the zinc phosphate oxidation inhibitor and zinc phosphate wear inhibitor comprises a mixture of zinc di(primary alkyl) dithiophosphate and zinc di(secondary alkyl) dithiophosphate in a weight ratio of 1/9 to 9/1.

11. The lubricating oil composition of claim 9, wherein the nitrogen-containing ashless dispersant is a succinimide dispersant which may be post-treated with ethylene carbonate or a borate compound.

12. The lubricating oil composition of claim 1, which further comprises a molybdenum complex of succinimide which may contain sulfur.

13. The lubricating oil composition of claim 1, wherein the oil of lubricating viscosity has a viscosity index of 120 to 160.

14. The lubricating oil composition of claim 1, which satisfies SAE viscosity grade of 0W20.

15. A method of making the lubricating oil composition of claim 1 comprising adding to an oil of lubricating viscosity the following additive components:
a molybdenum-containing friction modifier;
0.01 to 0.4 wt.%, in terms of calcium content, based on the total amount of the lubricating oil composition, of an overbased calcium salicylate having an alkyl group having an average carbon atom number in the range of 14 to 18, at least 60 mol.% of said alkyl group having a carbon atom number in the range of 14 to 18; and
0.01 to 0.4 wt.%, in terms of calcium content, based on the total amount of the lubricating oil composition, of at least one of the following calcium-containing detergent:
overbased calcium sulfonate having an alkyl group having an average carbon atom number in the range of 20 to 24, at least 60 mol.% of said alkyl group having a carbon atom number in the range of 20 to 24; and
overbased calcium salicylate having an alkyl group having an average carbon atom number in the range of 20 to 28, at least 60 mol.% of said alkyl group having a carbon atom number in the range of 20 to 28.

16. The method of claim 15, wherein the molybdenum-containing friction modifier comprises molybdenum dithiocarbamate.

17. The method of claim 15, wherein the calcium salicylate having an alkyl group having an average carbon atom number in the range of 14 to 18, at least 60 mol.% of said alkyl group having a carbon atom number in the range of 14 to 18 has an overbased degree of 1 to 4, and the calcium sulfonate having an alkyl group having an average carbon atom number in the range of 20 to 24, at least 60 mol.% of said alkyl group having a carbon atom number in the range of 20 to 24 and the calcium salicylate having an alkyl group having an average carbon atom number in the range of 20 to 28, at least 60 mol.% of said alkyl group having a carbon atom number in the range of 20 to 28 have an overbased degree of 6 to 24.

18. The method of claim 17, wherein the ratio of the overbased degree of the calcium sulfonate having an alkyl group having an average carbon atom number in the range of 20 to 24, at least 60 mol.% of said alkyl group having a carbon atom number in the range of 20 to 24 and the calcium salicylate having an alkyl group having an average carbon atom number in the range of 20 to 28, at least 60 mol.% of said alkyl group having a carbon atom number in the range of 20 to 28 to the calcium salicylate having an alkyl group having an average carbon atom number in the range of 14 to 18, at least 60 mol.% of said alkyl group having a carbon atom number in the range of 14 to 18 is in the range of 2 to 12.

19. The method of claim 15, wherein the at least one calcium-containing detergent is the calcium sulfonate having an alkyl group having an average carbon atom number in the range of 20 to 24, at least 60 mol.% of said alkyl group having a carbon atom number in the range of 20 to 24.

20. The method of claim 15, wherein the at least one calcium-containing detergent is the calcium salicylate having an alkyl group having an average carbon atom number in the range of 20 to 28, at least 60 mol.% of said alkyl group having a carbon atom number in the range of 20 to 28.

21. The method of claim 15, wherein the molybdenum-containing friction modifier is used in an amount of 0.01 to 0.15 wt.% in terms of molybdenum content in the lubricating oil composition.

22. The method of claim 15, further comprising adding a low overbased calcium sulfonate having an alkyl group having an average carbon atom number in the range of 14 to 24, at least 60 mol.% of said alkyl group having a carbon atom number in the range of 14 to 24 and having an overbased degree of 0.1 to 2.

23. The method of claim 15, further comprising adding a lubricating oil additive selected from the group consisting of a nitrogen-containing ashless dispersant, a zinc phosphate oxidation inhibitor, a zinc phosphate wear inhibitor, a phenolic oxidation inhibitor, and an amine oxidation inhibitor.

24. The method of claim 23, wherein each of the zinc phosphate oxidation inhibitor and zinc phosphate wear inhibitor comprises a mixture of zinc di(primary alkyl) dithiophosphate and zinc di(secondary alkyl) dithiophosphate in a weight ratio of 1/9 to 9/1.

25. The method of claim 23, wherein the nitrogen-containing ashless dispersant is a succinimide dispersant which may be post-treated with ethylene carbonate or a borate compound.

26. The method of claim 15, further comprising adding a molybdenum complex of succinimide which may contain sulfur.

27. The method of claim 15, wherein the oil of lubricating viscosity has a viscosity index of 120 to 160.

28. The method of claim 15, wherein the lubricating oil composition satisfies SAE viscosity grade of 0W20.

## Patentansprüche

1. Schmierölzusammensetzung für Verbrennungsmotoren, umfassend eine größere Menge eines Öls mit Schmierviskosität und eine kleinere Menge einer Zusatzmittelzusammensetzung, umfassend eine überbasierte metallhaltige Detergenszusammensetzung und einen molybdänhaltigen Reibungsmodifizierer;
worin die überbasierte metallhaltige Detergenszusammensetzung 0,01 bis 0,4 Gew.-%, nach Calciumgehalt, auf der Grundlage der Gesamtmenge der Schmierölzusammensetzung, eines Calciumsalicylats mit einer Alkylgruppe mit einer durchschnittlichen Kohlenstoffanzahl im Bereich von 14 bis 18 umfasst, wobei mindestens 60 Mol-% der Alkylgruppen eine Kohlenstoffanzahl im Bereich von 14 bis 18 haben, worin das Calciumsalicylat ein Gemisch aus einer Mehrzahl Calciumsalicylaten ist;
und 0,01 bis 0,4 Gew.-%, nach Calciumgehalt, auf der Grundlage der Gesamtmenge der Schmierölzusammensetzung, mindestens eines der folgenden calciumhaltigen Detergenzien:
Calciumsulfonat mit einer Alkylgruppe mit einer durchschnittlichen Kohlenstoffanzahl im Bereich von 20 bis 24, wobei mindestens 60 Mol-% der Alkylgruppen eine Kohlenstoffanzahl im Bereich von 20 bis 24 haben, wobei das Calciumsulfonat ein Gemisch aus einer Mehrzahl Calciumsulfonaten ist; und
Calciumsalicylat mit einer Alkylgruppe mit einer durchschnittlichen Kohlenstoffanzahl im Bereich von 20 bis 28, wobei mindestens 60 Mol-% der Alkylgruppen eine Kohlenstoffanzahl im Bereich von 20 bis 28 haben, wobei das Calciumsalicylat ein Gemisch aus einer Mehrzahl Calciumsalicylaten ist.

2. Schmierölzusammensetzung gemäß Anspruch 1, worin der molybdänhaltige Reibungsmodifizierer Molybdändithiocarbamat umfasst.

3. Schmierölzusammensetzung gemäß Anspruch 1, worin das Calciumsalicylat mit einer Alkylgruppe mit einer durchschnittlichen Kohlenstoffanzahl im Bereich von 14 bis 18, wobei mindestens 60 Mol-% der Alkylgruppen eine Kohlenstoffanzahl im Bereich von 14 bis 18 haben, einen Überbasierungsgrad von 1 bis 4 hat, und das Calciumsulfonat mit einer Alkylgruppe mit einer durchschnittlichen Kohlenstoffanzahl im Bereich von 20 bis 24, wobei mindestens 60 Mol-% der Alkylgruppen eine Kohlenstoffanzahl im Bereich von 20 bis 24 haben, und das Calciumsalicylat mit einer Alkylgruppe mit einer durchschnittlichen Kohlenstoffanzahl im Bereich von 20 bis 28, wobei mindestens 60 Mol-% der Alkylgruppen eine Kohlenstoffanzahl im Bereich von 20 bis 28 haben, einen Überbasierungsgrad von 6 bis 24 haben.

4. Schmierölzusammensetzung gemäß Anspruch 3, worin das Verhältnis des Überbasierungsgrads des Calciumsulfonats mit einer Alkylgruppe mit einer durchschnittlichen Kohlenstoffanzahl im Bereich von 20 bis 24, wobei mindestens 60 Mol-% der Alkylgruppen eine Kohlenstoffanzahl im Bereich von 20 bis 24 haben, und des Calciumsalicylats mit einer Alkylgruppe mit einer durchschnittlichen Kohlenstoffanzahl im Bereich von 20 bis 28, wobei mindestens 60 Mol-% der Alkylgruppen eine Kohlenstoffanzahl im Bereich von 20 bis 28 haben, zu dem des Calciumsalicylats mit einer Alkylgruppe mit einer durchschnittlichen Kohlenstoffanzahl im Bereich von 14 bis 18, wobei mindestens 60 Mol-% der Alkylgruppen eine Kohlenstoffanzahl im Bereich von 14 bis 18 haben, im Bereich von 2 bis 12 ist.

5. Schmierölzusammensetzung gemäß Anspruch 1, worin das überbasierte metallhaltige Detergens das Calciumsalicylat mit einer Alkylgruppe mit einer durchschnittlichen Kohlenstoffanzahl im Bereich von 14 bis 18 umfasst, wobei mindestens 60 Mol-% der Alkylgruppen eine Kohlenstoffanzahl im Bereich von 14 bis 18 haben, und das Calciumsulfonat mit einer Alkylgruppe mit einer durchschnittlichen Kohlenstoffanzahl im Bereich von 20 bis 24, wobei mindestens 60 Mol-% der Alkylgruppen eine Kohlenstoffanzahl im Bereich von 20 bis 24 haben, umfasst.

6. Schmierölzusammensetzung gemäß Anspruch 1, worin das überbasierte metallhaltige Detergens das Calciumsalicylat mit einer Alkylgruppe mit einer durchschnittlichen Kohlenstoffanzahl im Bereich von 14 bis 18 umfasst, wobei mindestens 60 Mol-% der Alkylgruppen eine Kohlenstoffanzahl im Bereich von 14 bis 18 haben, und das Calciumsalicylat mit einer Alkylgruppe mit einer durchschnittlichen Kohlenstoffanzahl im Bereich von 20 bis 28, wobei mindestens 60 Mol-% der Alkylgruppen eine Kohlenstoffanzahl im Bereich von 20 bis 28 haben, umfasst.

7. Schmierölzusammensetzung gemäß Anspruch 1, umfassend den molybdänhaltigen Reibungsmodifizierer in einer Menge von 0,01 bis 0,15 Gew.-%, nach Molybdängehalt in der Schmierölzusammensetzung.

8. Schmierölzusammensetzung gemäß Anspruch 1, das zudem ein leicht überbasiertes Calciumsulfonat mit einer Alkylgruppe mit einer durchschnittlichen Kohlenstoffanzahl im Bereich von 14 bis 24, wobei mindestens 60 Mol-% der Alkylgruppen eine Kohlenstoffanzahl im Bereich von 14 bis 24 haben, mit einem Überbasierungsgrad von 0,1 bis 2 umfasst.

9. Schmierölzusammensetzung gemäß Anspruch 1, zudem umfassend ein Schmierölzusatzmittel, ausgewählt aus der Gruppe stickstoffhaltiges aschefreies Dispergiermittel, Zinkphosphat-Oxydationshemmer, Zinkphosphat-Abriebhemmer, phenolischer Oxydationshemmer und Amin-Oxydationshemmer.

10. Schmierölzusammensetzung gemäß Anspruch 9, worin jedes aus dem Zinkphosphat-Oxydationshemmer und dem Zinkphosphat-Abriebhemmer, ein Gemisch aus Zinkdi(primäralkyl)dithiophosphat und Zinkdi(sekundäralkyl)-dithiophosphat in einem Gewichtsverhältnis von 1:9 bis 9:1 enthält.

11. Schmierölzusammensetzung gemäß Anspruch 9, worin das stickstoffhaltige aschefreie Dispergiermittel ein Bernsteinsäureimid-Dispergiermittel ist, das mit Ethylencarbonat oder einer Boratverbindung nachbehandelt sein kann.

12. Schmierölzusammensetzung gemäß Anspruch 1, das zudem einen Bernsteinsäureimid-Molybdänkomplex umfasst, der Schwefel enthalten kann.

13. Schmierölzusammensetzung gemäß Anspruch 1, worin das Öl mit Schmierviskosität eine Viskositätszahl von 120 bis 160 hat.

14. Schmierölzusammensetzung gemäß Anspruch 1, die einen SAE-Viskositätsgrad von 0W20 erfüllt.

15. Herstellungsverfahren für eine Schmierölzusammensetzung nach Anspruch 1, umfassend Zusetzen zu einem Öl mit Schmierviskosität der folgenden Zusatzmittelbestandteile
ein molybdänhaltiger Reibungsmodifizierer;
0,01 bis 0,4 Gew.-%, nach Calciumgehalt, auf der Grundlage der Gesamtmenge der Schmierölzusammensetzung, eines überbasierten Calciumsalicylats mit einer Alkylgruppe mit einer durchschnittlichen Kohlenstoffanzahl im Bereich von 14 bis 18 umfasst, wobei mindestens 60 Mol-% der Alkylgruppen eine Kohlenstoffanzahl im Bereich von 14 bis 18 haben; und
0,01 bis 0,4 Gew.-%, nach Calciumgehalt, auf der Grundlage der Gesamtmenge der Schmierölzusammensetzung, mindestens eines der folgenden calciumhaltigen Detergenzien:
überbasiertes Calciumsulfonat mit einer Alkylgruppe mit einer durchschnittlichen Kohlenstoffanzahl im Bereich von 20 bis 24, wobei mindestens 60 Mol-% der Alkylgruppen eine Kohlenstoffanzahl im Bereich von 20 bis 24 haben; und
überbasiertes Calciumsalicylat mit einer Alkylgruppe mit einer durchschnittlichen Kohlenstoffanzahl im Bereich von 20 bis 28, wobei mindestens 60 Mol-% der Alkylgruppen eine Kohlenstoffanzahl im Bereich von 20 bis 28 haben.

16. Verfahren gemäß Anspruch 15, worin der molybdänhaltige Reibungsmodifizierer Molybdändithiocarbamat umfasst.

17. Verfahren gemäß Anspruch 15, worin das Calciumsalicylat mit einer Alkylgruppe mit einer durchschnittlichen Kohlenstoffanzahl im Bereich von 14 bis 18, wobei mindestens 60 Mol-% der Alkylgruppen eine Kohlenstoffanzahl im Bereich von 14 bis 18 haben, einen Überbasierungsgrad von 1 bis 4 hat, und das Calciumsulfonat mit einer Alkylgruppe mit einer durchschnittlichen Kohlenstoffanzahl im Bereich von 20 bis 24, wobei mindestens 60 Mol-% der Alkylgruppen eine Kohlenstoffanzahl im Bereich von 20 bis 24 haben, und das Calciumsalicylat mit einer Alkylgruppe mit einer durchschnittlichen Kohlenstoffanzahl im Bereich von 20 bis 28, wobei mindestens 60 Mol-% der Alkylgruppen eine Kohlenstoffanzahl im Bereich von 20 bis 28 haben, einen Überbasierungsgrad von 6 bis 24 haben.

18. Verfahren gemäß Anspruch 17, worin das Verhältnis des Überbasierungsgrads des Calciumsulfonats mit einer Alkylgruppe mit einer durchschnittlichen Kohlenstoffanzahl im Bereich von 20 bis 24, wobei mindestens 60 Mol-% der Alkylgruppen eine Kohlenstoffanzahl im Bereich von 20 bis 24 haben, und des Calciumsalicylats mit einer Alkylgruppe mit einer durchschnittlichen Kohlenstoffanzahl im Bereich von 20 bis 28, wobei mindestens 60 Mol-% der Alkylgruppen eine Kohlenstoffanzahl im Bereich von 20 bis 28 haben, zu dem des Calciumsalicylats mit einer Alkylgruppe mit einer durchschnittlichen Kohlenstoffanzahl im Bereich von 14 bis 18, wobei mindestens 60 Mol-% der Alkylgruppen eine Kohlenstoffanzahl im Bereich von 14 bis 18 haben, im Bereich von 2 bis 12 ist.

19. Verfahren gemäß Anspruch 15, worin das mindestens ein calciumhaltige Detergens das Calciumsulfonat ist mit einer Alkylgruppe mit einer durchschnittlichen Kohlenstoffanzahl im Bereich von 20 bis 24, wobei mindestens 60 Mol-% der Alkylgruppen eine Kohlenstoffanzahl im Bereich von 20 bis 24 haben.

20. Verfahren gemäß Anspruch 15, worin das mindestens ein calciumhaltige Detergens das Calciumsalicylat ist mit einer Alkylgruppe mit einer durchschnittlichen Kohlenstoffanzahl im Bereich von 20 bis 28, wobei mindestens 60 Mol-% der Alkylgruppen eine Kohlenstoffanzahl im Bereich von 20 bis 28 haben.

21. Verfahren gemäß Anspruch 15, worin der molybdänhaltige Reibungsmodifizierer in einer Menge von 0,01 bis 0,15 Gew.-%, nach Molybdängehalt in der Schmierölzusammensetzung, verwendet wird.

22. Verfahren gemäß Anspruch 15, zudem umfassend Zusetzen eines leicht überbasierten Calciumsulfonats mit einer Alkylgruppe mit einer durchschnittlichen Kohlenstoffanzahl im Bereich von 14 bis 24, wobei mindestens 60 Mol-% der Alkylgruppen eine Kohlenstoffanzahl im Bereich von 14 bis 24 haben, mit einem Überbasierungsgrad von 0,1 bis 2.

23. Verfahren gemäß Anspruch 15, zudem umfassend ein Schmierölzusatzmittel, ausgewählt aus der Gruppe stickstoffhaltiges aschefreies Dispergiermittel, Zinkphosphat-Oxydationshemmer, Zinkphosphat-Abriebhemmer, phenolischer Oxydationshemmer und Amin-Oxydationshemmer.

24. Verfahren gemäß Anspruch 23, worin jedes aus dem Zinkphosphat-Oxydationshemmer und dem Zinkphosphat-Abriebhemmer, ein Gemisch aus Zinkdi(primäralkyl)dithiophosphat und Zinkdi(sekundäralkyl)dithiophosphat in einem Gewichtsverhältnis von 1:9 bis 9:1 enthält.

25. Verfahren gemäß Anspruch 23, worin das stickstoffhaltige aschefreie Dispergiermittel ein Bernsteinsäureimid-Dispergiermittel ist, das mit Ethylencarbonat oder einer Boratverbindung nachbehandelt sein kann.

26. Verfahren gemäß Anspruch 15, zudem umfassend einen Bernsteinsäureimid-Molybdänkomplex, der Schwefel enthalten kann.

27. Verfahren gemäß Anspruch 15, worin das Öl mit Schmierviskosität eine Viskositätszahl von 120 bis 160 hat.

28. Verfahren gemäß Anspruch 15, worin die Schmierölzusammensetzung die einen SAE-Viskositätsgrad von 0W20 erfüllt.

## Revendications

1. Composition d'huile lubrifiante pour moteur à combustion interne qui comprend une quantité majeure d'une huile à viscosité lubrifiante et une quantité mineure d'une composition d'additifs comprenant une composition superbasée de détergent contenant un métal et un modificateur de friction comprenant du molybdène ;
dans laquelle la composition superbasée de détergent contenant un métal comprend de 0,01 à 0,4 pour cent en poids, en termes du contenu en calcium, à la base du poids total de la composition d'huile lubrifiante, d'un salicylate de calcium ayant un groupe alkyle avec un nombre moyen en atomes de carbone dans l'intervalle de 14 à 18, au moins 60 pour cent molaire dudit groupe alkyle ayant un nombre moyen en atomes de carbone dans l'intervalle de 14 à 18, dans laquelle le salicylate de calcium est un mélange d'une pluralité de salicylates de calcium ;
et de 0,01 à 0,4 pour cent en poids, en termes du contenu en calcium, à la base du poids total de la composition d'huile lubrifiante, d'au moins un parmi les détergents comprenant du calcium suivants :
du sulfonate de calcium ayant un groupe alkyle avec un nombre moyen en atomes de carbone dans l'intervalle de 20 à 24, au moins 60 pour cent molaire dudit groupe alkyle ayant un nombre moyen en atomes de carbone dans l'intervalle de 20 à 24, dans laquelle le sulfonate de calcium est un mélange d'une pluralité de sulfonates de calcium ; et
du salicylate de calcium ayant un groupe alkyle avec un nombre moyen en atomes de carbone dans l'intervalle de 20 à 28, au moins 60 pour cent molaire dudit groupe alkyle ayant un nombre moyen en atomes de carbone dans l'intervalle de 20 à 28, dans laquelle le salicylate de calcium est un mélange d'une pluralité de salicylates de calcium.

2. Composition d'huile lubrifiante selon la revendication 1, dans laquelle le modificateur de friction comprenant du molybdène comprend du dithiocarbamate de molybdène.

3. Composition d'huile lubrifiante selon la revendication 1, dans laquelle le salicylate de calcium ayant un groupe alkyle avec un nombre moyen en atomes de carbone dans l'intervalle de 14 à 18, au moins 60 pour cent molaire dudit groupe alkyle ayant un nombre moyen en atomes de carbone dans l'intervalle de 14 à 18, a un degré de superbasicité de 1 à 4, et le sulfonate de calcium ayant un groupe alkyle avec un nombre moyen en atomes de carbone dans l'intervalle de 20 à 24, au moins 60 pour cent molaire dudit groupe alkyle ayant un nombre moyen en atomes de carbone dans l'intervalle de 20 à 24, et le salicylate de calcium ayant un groupe alkyle avec un nombre moyen en atomes de carbone dans l'intervalle de 20 à 28, au moins 60 pour cent molaire dudit groupe alkyle ayant un nombre moyen en atomes de carbone dans l'intervalle de 20 à 28, ont un degré de superbasicité de 6 à 24.

4. Composition d'huile lubrifiante selon la revendication 3, dans laquelle le rapport du degré de superbasicité du sulfonate de calcium ayant un groupe alkyle avec un nombre moyen en atomes de carbone dans l'intervalle de 20 à 24, au moins 60 pour cent molaire dudit groupe alkyle ayant un nombre moyen en atomes de carbone dans l'intervalle de 20 à 24, et du salicylate de calcium ayant un groupe alkyle avec un nombre moyen en atomes de carbone dans l'intervalle de 20 à 28, au moins 60 pour cent molaire dudit groupe alkyle ayant un nombre moyen en atomes de carbone dans salicylate de calcium ayant un groupe alkyle avec un nombre moyen en atomes de carbone dans l'intervalle de 20 à 28, par rapport à celui du salicylate de calcium ayant un groupe alkyle avec un nombre moyen en atomes de carbone dans l'intervalle de 14 à 18, au moins 60 pour cent molaire dudit groupe alkyle ayant un nombre moyen en atomes de carbone dans l'intervalle de 14 à 18, est dans l'intervalle de 2 à 12.

5. Composition d'huile lubrifiante selon la revendication 1, dans laquelle la composition superbasée de détergent contenant un métal comprend le salicylate de calcium ayant un groupe alkyle avec un nombre moyen en atomes de carbone dans l'intervalle de 14 à 18, au moins 60 pour cent molaire dudit groupe alkyle ayant un nombre moyen en atomes de carbone dans l'intervalle de 14 à 18, et le sulfonate de calcium ayant un groupe alkyle avec un nombre moyen en atomes de carbone dans l'intervalle de 20 à 24, au moins 60 pour cent molaire dudit groupe alkyle ayant un nombre moyen en atomes de carbone dans l'intervalle de 20 à 24.

6. Composition d'huile lubrifiante selon la revendication 1, dans laquelle la composition superbasée de détergent contenant un métal comprend le salicylate de calcium ayant un groupe alkyle avec un nombre moyen en atomes de carbone dans l'intervalle de 14 à 18, au moins 60 pour cent molaire dudit groupe alkyle ayant un nombre moyen en atomes de carbone dans l'intervalle de 14 à 18, et le salicylate de calcium ayant un groupe alkyle avec un nombre moyen en atomes de carbone dans l'intervalle de 20 à 28, au moins 60 pour cent molaire dudit groupe alkyle ayant un nombre moyen en atomes de carbone dans l'intervalle de 20 à 28.

7. Composition d'huile lubrifiante selon la revendication 1, qui comprend le modificateur de friction comprenant du molybdène en une quantité de 0,01 à 0,15 pour cent en poids en termes du contenu en molybdène dans la composition d'huile lubrifiante.

8. Composition d'huile lubrifiante selon la revendication 1, qui comprend en plus un sulfonate de calcium légèrement superbasé ayant un groupe alkyle avec un nombre moyen en atomes de carbone dans l'intervalle de 14 à 24, au moins 60 pour cent molaire dudit groupe alkyle ayant un nombre moyen en atomes de carbone dans l'intervalle de 14 à 24, et ayant un degré de superbasicité de 0,1 à 2.

9. Composition d'huile lubrifiante selon la revendication 1, qui comprend en plus un additif d'huile lubrifiante sélectionné parmi le groupe constitué en un dispersant libre de cendres contenant de l'azote, un inhibiteur d'oxydation à la base de phosphate de zinc, un inhibiteur d'usure à la base de phosphate de zinc, un inhibiteur d'oxydation phénolique, et un inhibiteur d'oxydation à la base d'amine.

10. Composition d'huile lubrifiante selon la revendication 9, dans laquelle chacun parmi l'inhibiteur d'oxydation à la base de phosphate de zinc et l'inhibiteur d'usure à la base de phosphate de zinc comprend un mélange de di(alkyle primaire)dithiophosphate de zinc et di(alkyle secondaire)dithiophosphate en un rapport en poids de 1:9 à 9:1.

11. Composition d'huile lubrifiante selon la revendication 9, dans laquelle le dispersant libre de cendres contenant de l'azote est un dispersant à la base de succinimide qui peut être post-traité avec du carbonate d'éthylène ou un composé borate..

12. Composition d'huile lubrifiante selon la revendication 1, qui comprend en plus un complexe succinimide du molybdène qui peut contenir du soufre.

13. Composition d'huile lubrifiante selon la revendication 1, dans laquelle l'huile à viscosité lubrifiante a un indice de viscosité de 120 à 160.

14. Composition d'huile lubrifiante selon la revendication 1, qui satisfait un degré de viscosité SAE de 0W20.

15. Un procédé pour préparer la composition d'huile lubrifiante selon la revendication 1, comprenant ajouter à une huile à viscosité lubrifiante les composantes d'additifs suivantes :
un modificateur de friction comprenant du molybdène ;
de 0,01 à 0,4 pour cent en poids, en termes du contenu en calcium, à la base du poids total de la composition d'huile lubrifiante, d'un salicylate de calcium ayant un groupe alkyle avec un nombre moyen en atomes de carbone dans l'intervalle de 14 à 18, au moins 60 pour cent molaire dudit groupe alkyle ayant un nombre moyen en atomes de carbone dans l'intervalle de 14 à 18 ; et
de 0,01 à 0,4 pour cent en poids, en termes du contenu en calcium, à la base du poids total de la composition d'huile lubrifiante, d'au moins un parmi les détergents comprenant du calcium suivants :
du sulfonate de calcium ayant un groupe alkyle avec un nombre moyen en atomes de carbone dans l'intervalle de 20 à 24, au moins 60 pour cent molaire dudit groupe alkyle ayant un nombre moyen en atomes de carbone dans l'intervalle de 20 à 24 ; et
du salicylate de calcium ayant un groupe alkyle avec un nombre moyen en atomes de carbone dans l'intervalle de 20 à 28, au moins 60 pour cent molaire dudit groupe alkyle ayant un nombre moyen en atomes de carbone dans l'intervalle de 20 à 28.

16. Procédé selon la revendication 15, dans lequel le modificateur de friction comprenant du molybdène comprend du dithiocarbamate de molybdène.

17. Procédé selon la revendication 15, dans lequel le salicylate de calcium ayant un groupe alkyle avec un nombre moyen en atomes de carbone dans l'intervalle de 14 à 18, au moins 60 pour cent molaire dudit groupe alkyle ayant un nombre moyen en atomes de carbone dans l'intervalle de 14 à 18, a un degré de superbasicité de 1 à 4, et le sulfonate de calcium ayant un groupe alkyle avec un nombre moyen en atomes de carbone dans l'intervalle de 20 à 24, au moins 60 pour cent molaire dudit groupe alkyle ayant un nombre moyen en atomes de carbone dans l'intervalle de 20 à 24, et le salicylate de calcium ayant un groupe alkyle avec un nombre moyen en atomes de carbone dans l'intervalle de 20 à 28, au moins 60 pour cent molaire dudit groupe alkyle ayant un nombre moyen en atomes de carbone dans l'intervalle de 20 à 28, ont un degré de superbasicité de 6 à 24.

18. Procédé selon la revendication 17, dans lequel le rapport du degré de superbasicité du sulfonate de calcium ayant un groupe alkyle avec un nombre moyen en atomes de carbone dans l'intervalle de 20 à 24, au moins 60 pour cent molaire dudit groupe alkyle ayant un nombre moyen en atomes de carbone dans l'intervalle de 20 à 24, et du salicylate de calcium ayant un groupe alkyle avec un nombre moyen en atomes de carbone dans l'intervalle de 20 à 28, au moins 60 pour cent molaire dudit groupe alkyle ayant un nombre moyen en atomes de carbone dans salicylate de calcium ayant un groupe alkyle avec un nombre moyen en atomes de carbone dans l'intervalle de 20 à 28, par rapport à celui du salicylate de calcium ayant un groupe alkyle avec un nombre moyen en atomes de carbone dans l'intervalle de 14 à 18, au moins 60 pour cent molaire dudit groupe alkyle ayant un nombre moyen en atomes de carbone dans l'intervalle de 14 à 18, est dans l'intervalle de 2 à 12.

19. Procédé selon la revendication 15, dans lequel l'au moins un détergent contenant un calcium est le sulfonate de calcium ayant un groupe alkyle avec un nombre moyen en atomes de carbone dans l'intervalle de 20 à 24, au moins 60 pour cent molaire dudit groupe alkyle ayant un nombre moyen en atomes de carbone dans l'intervalle de 20 à 24.

20. Procédé selon la revendication 15, dans lequel l'au moins un détergent contenant un calcium est le salicylate de calcium ayant un groupe alkyle avec un nombre moyen en atomes de carbone dans l'intervalle de 20 à 28, au moins 60 pour cent molaire dudit groupe alkyle ayant un nombre moyen en atomes de carbone dans l'intervalle de 20 à 28.

21. Procédé selon la revendication 15, dans lequel le modificateur de friction comprenant du molybdène est utilisé en une quantité de 0,01 à 0,15 pour cent en poids en termes du contenu en molybdène dans la composition d'huile lubrifiante.

22. Procédé selon la revendication 15, comprenant en plus ajouter un sulfonate de calcium légèrement superbasé ayant un groupe alkyle avec un nombre moyen en atomes de carbone dans l'intervalle de 14 à 24, au moins 60 pour cent molaire dudit groupe alkyle ayant un nombre moyen en atomes de carbone dans l'intervalle de 14 à 24, et ayant un degré de superbasicité de 0,1 à 2.

23. Procédé selon la revendication 15, comprenant en plus ajouter un additif d'huile lubrifiante sélectionné parmi le groupe constitué en un dispersant libre de cendres contenant de l'azote, un inhibiteur d'oxydation à la base de phosphate de zinc, un inhibiteur d'usure à la base de phosphate de zinc, un inhibiteur d'oxydation phénolique, et un inhibiteur d'oxydation à la base d'amine.

24. Procédé selon la revendication 23, dans lequel chacun parmi l'inhibiteur d'oxydation à la base de phosphate de zinc et l'inhibiteur d'usure à la base de phosphate de zinc comprend un mélange de di(alkyle primaire)dithiophosphate de zinc et di(alkyle secondaire)dithiophosphate en un rapport en poids de 1:9 à 9:1.

25. Procédé selon la revendication 23, dans lequel le dispersant libre de cendres contenant de l'azote est un dispersant à la base de succinimide qui peut être post-traité avec du carbonate d'éthylène ou un composé borate.

26. Procédé selon la revendication 15, comprenant en plus ajouter un complexe succinimide du molybdène qui peut contenir du soufre.

27. Procédé selon la revendication 15, dans lequel l'huile à viscosité lubrifiante a un indice de viscosité de 120 à 160.

28. Procédé selon la revendication 15, dans lequel la composition d'huile lubrifiante satisfait un degré de viscosité SAE de 0W20.
